

1

3,708,257

**PROCESS FOR THE DYEING OF TEXTILE MATERIAL MADE FROM MIXTURES OF POLYESTER AND CELLULOSIC FIBERS**

Rudolf Lowenfeld, Buchschlag, and Uwe Kosubek, Offenbach, Main, Germany, assignors to Farbwerke Hoechst Aktiengesellschaft vormals Meister Lucius & Bruning, Frankfurt am Main, Germany

No Drawing. Filed Oct. 27, 1970, Ser. No. 84,544

Claims priority, application Germany, Oct. 29, 1969,  
P 19 54 294.0  
Int. Cl. D06p 3/82

U.S. Cl. 8—21 C

6 Claims

**ABSTRACT OF THE DISCLOSURE**

Process for the dyeing of textile material consisting of mixtures of polyester and cellulosic fibers, wherein said textile material is impregnated with an alkaline solution containing a substantive coupling component, as well as a wetting or dispersing agent, dried, subsequently treated with an acid aqueous solution containing a diazotized aromatic amine and a compound having an acidic reaction, dried, impregnated with at least one disperse dyestuff and then subjected to a heat-treatment.

It is known that textile material made from mixtures of polyester and cellulosic fibers can be dyed fast shades by using disperse dyestuffs and water-insoluble azo dyestuffs, the latter being produced on the fiber. The procedure is as follows: the polyester fiber portion of the goods is first dyed with disperse dyestuffs, either at boiling temperature in the presence of dyeing accelerators, or under the conditions of high-temperature dyeing, or according to the so-called Thermosol process; subsequently the water-insoluble azo dyestuff is produced on the cellulosic fiber portion by impregnating the textiles with a coupling component and thereafter developing the dye with a diazotized aromatic amine.

In many cases, this process yields dyeings of useful quality. In other cases, especially with the production of blue, water-insoluble azo dyestuffs on the cellulosic fiber portion of the mixed fabrics, dyeings result the fastness of which to rubbing does not comply with the practical requirements.

The cause of the deficient fastness to rubbing may be seen in the fact that during development a certain portion of the water-insoluble azo dyestuff is formed in the surface zone of the polyester fiber portion and is not removed during the following washing process. This dyestuff which sticks to the polyester fiber portion is rubbed off on abrasion of the dyed fabric by means of undyed material and renders the dyeing substantially useless.

This invention is based on the observation that the aforementioned disadvantages in the dyeing of textile material made from mixtures of polyester and cellulosic fibers can be overcome by impregnating said textile material with alkaline solutions containing a coupling component as well as wetting or dispersing agents, drying and subsequently treating the material with aqueous solutions of acidic agents which contain a diazotized aromatic amine and a compound having an acidic reaction, drying, impregnating with at least one disperse dyestuff and then subjecting it to a heat-treatment.

The process of the invention is carried out as follows: the textile material, for example mixed fabrics made from polyester and cellulosic fibers, is impregnated with an alkaline solution containing a coupling component, as well as wetting or dispersing agents, squeezed and then dried. Thereby, the alkali concentration of the impreg-

2

nation bath should be kept at such a high level which ensures non-precipitation of the coupling component during impregnation. Subsequently, the textile material is impregnated with a solution containing compounds having an acidic reaction, a diazotized primary aromatic amine, as well as, if desired or required, a dispersing agent. The concentration of the compounds having an acidic reaction should be at a level which ensures neutralization of the alkali applied to the textile material together with the coupling component in the alkaline impregnation process, and the material to be dyed should have a pH-value of from 4 to 7. Corresponding to the coupling capability of the diazotized aromatic amine used, the goods are subsequently treated in a neutral or alkaline cold or warm bath in order to complete coupling.

After dyestuff formation, the material is subjected to an alkaline after-treatment in usual manner at boiling temperatures, rinsed and dried. Subsequently, it is impregnated with the aqueous suspension of at least one disperse dyestuff, squeezed, dried and the textile material is subjected to a heat-treatment in the range of from about 170° to 220° C. This heat-treatment may be carried out by means of hot air or contact heat. In the process of the invention, remainders of the insoluble azo dyestuff, which had not been washed out before, and the disperse dyestuff applied at last, migrate into the interior of the polyester fiber during the heat treatment and are there fixed. Finally, the material is subjected to an alkaline after-treatment, rinsed and dried.

On this method, the azo dyestuff is obtained in full yield and clearness. The dyeings obtained have a better fastness to rubbing than dyeings with which first the disperse dyestuff was fixed separately by heat-treatment on the polyester fiber portion and the water-insoluble azo dyestuff was subsequently produced on the cellulosic fiber portion in known manner.

Examples of the textile material to be dyed are mixtures containing between 25% of polyester and 75% of cellulosic fibers and 70% of polyester and 30% of cellulosic fibers.

Suitable polyester fibers in the blend are fibers made from aromatic polyesters, for example from terephthalic acid or diphenyl-4,4'-dicarboxylic acid and alkane diols or 1,4-cyclohexane-di-methanol, as well as those consisting of triacetyl cellulose. The cellulosic fiber portion may be of natural or regenerated origin.

Examples of the coupling components to be used in the process of the invention are especially aromatic o-hydroxycarboxylic acid arylamides or acylacetic acid arylamides, 6-bromo- or 6-alkoxy-2,3-hydroxynaphthoic acid arylamides or acetoacetic acid arylamides which have a low to medium substantivity towards cellulosic fibers. When suitable impregnation equipment is used, for example one with a small-sized bath tank, coupling components having a high substantivity towards cellulosic fibers may also be used, for example the condensation products from 2,3-hydroxynaphthoic acid and polynuclear, isocyclic and heterocyclic amines, for example aminonaphthalenes, aminocarbazoles or aminodiphenylene oxides.

As diazotized primary aromatic amines mono- or di- amines may be used, for example diazotized chloroanilines, dichloroanilines, chlorotoluidines, chloroanisidines, nitranilines, nitrotoluidines, nitroanisidines, nitroxydines, nitrophenetidines, cyanotoluidines, cyanoanisidines, aminobenzene sulfonic acid amides, aminobenzene carboxylic acid amides, aminophenyl-alkylsulfones, aminophenyl-arylsulfones or aminophenyl-aralkylsulfones, aminodiphenyl ethers, trifluoromethylanilines, monoacylated phenylenediamines, aminoazobenzenes, as well as tetra-4,4'-diamino-diphenyls.

Suitable wetting or dispersing agents in the alkaline impregnation bath are condensation products from high-molecular fatty acids and protein degradation products, condensation products from high-molecular fatty acids and aminoalkyl sulfonic acids, condensation products from formaldehyde and naphthalene sulfonic acids, Monopol brilliant oil as well as purified sulfite-cellulose waste liquor.

The compounds having an acidic reaction may be organic acids, for example acetic acid, formic acid, propionic acid, glycolic acid, tartaric acid or citric acid, complex chromium salts of the acetic acid which have weakly acidic reaction or other salts having an acidic reaction, for example monosodium phosphate or aluminium sulfate.

As disperse dyestuffs there may be used such dyestuffs which are suitable for the Thermosol process on account of their thermal properties, i.e. dyestuffs which are capable of dyeing polyester fibers at temperatures in the range of from 170° to 220° C. and which do not soil the dyeing equipment on account of high volatility. Suitable disperse dyestuffs of the azo and anthraquinone series are described in Colour-Index, second edition 1959, vol. 1, p. 1659-1742 and Supplement 1963, p. S 179-224, as well as in the corresponding additions and amendments, No. 1 (September 1963) to No. 23 (April 1969).

The process of the invention may be carried out continuously or semi-continuously.

The following example illustrates the invention.

passed into water of the temperature of 60° C., subsequently subjected to alkaline washing and dried. The material was then impregnated by means of an aqueous suspension of 40 g. of the disperse dyestuff: aniline → 1-(2',3'-hydroxynaphthoylamino)-4-methoxybenzene per liter of water, squeezed in such a way that the liquor uptake amounted to 60% of the dry weight of the material, dried and passed through a fixing chamber or over hot rollers in such a way that the goods were heated for 30-60 seconds to 180° C.-210° C.

Finally, the fabric was after-treated, at boiling temperature, with a solution containing 2 g. of a 30% reaction product of about 10 mols of ethylene oxide with 1 mol of nonylphenol, 2 ml. of a 25% solution of the sodium salt of nitrilotriacetic acid and 2 g. of sodium carbonate per liter of water and then rinsed hot and cold. The after-treatment of the dyed fabric might also be carried out at 60° C. or 95° C. in a bath containing, per liter of water, 3 g. of a mixture of 63% perchloroethylene, 17% of a reaction product of about 10 mols of ethylene oxide with 1 mol of nonylphenol and 20% of isopropylalcohol, together with 2 g. of a 25% solution of the sodium salt of nitrilo-triaceic acid. An intense red dyeing having good fastness properties was obtained.

The following table lists further coupling components, diazo components and disperse dyestuffs that may be used according to the process of the invention, as well as the shades obtainable therefrom on mixed fabrics containing 67% of polyethylene terephthalate fibers and 33% of cotton.

| Coupling component                                             | Diazo component                                               | Disperse dyestuff                                                                                                                                                                                                                            | Shade          |
|----------------------------------------------------------------|---------------------------------------------------------------|----------------------------------------------------------------------------------------------------------------------------------------------------------------------------------------------------------------------------------------------|----------------|
| 1-(2',3'-hydroxynaphthoylamino)-2-methoxybenzene.              | 1-amino-3-chlorobenzene                                       | 1-amino-4-phenylazonaphthalene → phenol                                                                                                                                                                                                      | Orange.        |
| 2,3-hydroxynaphthoylaminobenzene                               | 1-amino-2-nitro-4-chlorobenzene                               | 1-amino-4-nitrobenzene → 3-methyl-N,N-bis-β-hydroxyethylaniline.                                                                                                                                                                             | Red.           |
| Do                                                             | 1-amino-4-chloro-2-trifluoromethylbenzene                     | Aniline → 1-2',3-(hydroxynaphthoylamino)-4-methoxybenzene plus 1-amino-4-nitrobenzene → 3-methyl-N,N-bis-β-hydroxyethylaniline.                                                                                                              | Yellowish red. |
| Do                                                             | 1-amino-2-methoxy-4-nitrobenzene                              | 1-amino-2-cyano-4-nitrobenzene → N,N-bis-(β-acetoxyethyl)-aniline.                                                                                                                                                                           | Bluish red.    |
| Do                                                             | o-aminoazotoluene                                             | do                                                                                                                                                                                                                                           | Scarlet.       |
| 1-(2',3'-hydroxynaphthoylamino)-2-methoxybenzene.              | 1-amino-2-methyl-5-chlorobenzene                              | 1-amino-2-cyano-4-nitrobenzene → N-β-cyanoethyl-N-β-carbomethoxyethylaniline.                                                                                                                                                                | Red.           |
| Do                                                             | do                                                            | do                                                                                                                                                                                                                                           | Red.           |
| 1-acetoacetyl amino-2,5-dimethoxy-4-chlorobenzene.             | 1-amino-2-methyl-4-chlorobenzene                              | 1-amino-3-nitrobenzene → 4-hydroxy-1-methylcarbo-styryl.                                                                                                                                                                                     | Yellow.        |
| Do                                                             | 1-amino-2-chlorobenzene                                       | do                                                                                                                                                                                                                                           | Do.            |
| 4,4'-bis-acetoacetylarnino-3,3'-dimethyl-diphenyl.             | do                                                            | do                                                                                                                                                                                                                                           | Do.            |
| 1-(2',3'-hydroxynaphthoylamino)-2-methyl-4-chlorobenzene.      | 1-amino-2-methyl-5-chlorobenzene                              | 1-amino-2-cyano-4-nitrobenzene → N-β-cyanoethyl-N-β-carbomethoxyethylaniline.                                                                                                                                                                | Red.           |
| 2,3-hydroxynaphthoylaminobenzene                               | 4-amino-4'-methoxydiphenylamine                               | 1,5-dihydroxy-4,8-diamino-bromoanthraquinone.                                                                                                                                                                                                | Blue.          |
| Do                                                             | 4-amino-2,5-dimethoxy-2',6'-dichloro-4'-nitro-1,1-azobenzene. | 1-amino-2-bromo-4,6-dinitrobenzene → 2-ethoxy-5-acetylamino-N,N-bis-(β-acetoxyethyl)-aniline plus 1-amino-3-nitrobenzene → 4-hydroxy-1-methylcarbo-styryl plus 1-amino-2-cyano-4-nitrobenzene → N-β-cyanoethyl-N-β-carbomethoxyethylaniline. | Navy blue.     |
| 1-(2',3'-hydroxynaphthoylamino)-2,4-dimethoxy-5-chlorobenzene. | do                                                            | 1-amino-2-bromo-4,6-dinitrobenzene → 2-ethoxy-5-acetylamino-N,N-bis-(β-acetoxyethyl)-aniline plus 1-amino-3-nitrobenzene → 4-hydroxy-1-methylcarbo-styryl plus 1-amino-2-cyano-4-nitrobenzene → N-β-cyanoethyl-N-β-carbomethoxyethylaniline. | Do.            |
| 2,3-hydroxynaphthoylaminobenzene                               | 1-amino-4-benzoylamino-2,5-diethoxy-benzene.                  | 1,8-dihydroxy-4,5-diaminoanthraquinone.                                                                                                                                                                                                      | Blue.          |

### EXAMPLE

A mixed fabric consisting of 67% of polyethylene terephthalate fibers and 33% of cotton was impregnated with a solution containing per liter of water 14 g. of 2,3-hydroxynaphthoylaminobenzene dissolved in 14 ml. of 32.5% sodium hydroxide solution and water of the temperature of 90° C., as well as 4 g. of a wetting agent of the type of the oleic sulfonates. The fabric was then squeezed in such a way that the liquor uptake amounted to 60% of the dry weight of the material, dried and impregnated with a solution containing per liter of water 7.6 g. of diazotized 1-amino-2-nitrobenzene, 20 ml. of 50% acetic acid and 15 g. of sodium acetate, and once more squeezed in such a way that the liquor uptake amounted to 60% of the dry weight of the material. After an air passage of about 60 seconds, the goods were

What we claim is:

1. A process for the dyeing of textile material consisting of mixtures of polyester and cellulosic fibers, wherein said textile material is impregnated with an alkaline solution containing a substantive coupling component, as well as a wetting or dispersing agent, dried, subsequently treated with an acid aqueous solution containing a diazotized aromatic amine and a compound having an acidic reaction, dried, impregnated with at least one disperse dyestuff and then subjected to a heat-treatment.

2. A process as claimed in claim 1, wherein the coupling component is an aromatic or heterocyclic o-hydroxycarboxylic acid arylamide or an acetoacetic acid arylamide.

3. A process as claimed in claim 1, wherein a diazo compound of the benzene, diphenyl or azobenzene series is used.

4. A process as claimed in claim 1, wherein a disperse dyestuff of the azo or anthraquinone series is used.

5. A process as claimed in claim 1, wherein the acid impregnation is carried out at a pH in the range of from 4 to 7.

6. A process as claimed in claim 1, wherein the heat-treatment is effected at a temperature within the range of from 170° to 220° C.

## OTHER REFERENCES

Fortess et al., Amer. Dyestuff Reporter, May 1963, pp. 402-409.

5 Schmidlin, Preparation and Dyeing of Synthetic Fibers, Publ. April 1963, by Chapman & Hall Ltd., pp. 264-274.

W. J. Wygand, Amer. Dyestuff Reporter, December 1964, pp. 106-108.

DuPont Bulletin, D-238, March 1970, p. 10.

10 GEORGE F. LESMES, Primary Examiner

T. J. HERBERT, JR., Assistant Examiner

U.S. CL. X.R.

8-26, 46

## References Cited

## UNITED STATES PATENTS

|           |         |                    |        |    |
|-----------|---------|--------------------|--------|----|
| 3,416,873 | 12/1968 | Fono et al. -----  | 8-21 C | 15 |
| 3,100,132 | 8/1963  | Jenny et al. ----- | 8-39   |    |